

## UNITED STATES PATENT OFFICE

BENJAMIN L. JOHNSON, OF GARFIELD, UTAH

## CONCENTRATION OF ORES

No Drawing.

Application filed October 31, 1928. Serial No. 316,368.

This invention relates to the concentration of ores, minerals and the like by flotation, and has for its object the provision of certain improvements in flotation processes, and more particularly the froth flotation process.

The present invention is based upon the discovery that tetrathio diphospho organic compounds are effective flotation agents. I have found that these compounds, in which two molecules of an organic phosphorus and sulphur containing compound are made to combine into a single molecule, with two phosphorus atoms bonded through two intervening and linked sulphur atoms, have a marked selective action on the sulphide minerals as distinguished from gangue minerals; and when used in a flotation process, float the sulphide minerals readily with an attendant high recovery of the metal values.

I have also found that smaller amounts of these tetrathio diphospho organic compounds are needed to produce equivalent or better results in the flotation operation than other organic flotation agents heretofore generally used.

My investigations indicate that certain of the tetrathio diphospho organic compounds have insufficient frothing power to constitute a complete agent in froth-flotation, so that an appropriate frothing agent, such as pine oil, cresylic acid or the like, may be employed in conjunction therewith, in carrying out such froth-flotation operation.

The flotation agent which is typical of these tetrathio diphospho organic compounds may be conveniently made by adding diethyl dithio phosphoric acid, or its metallic salt, during continuous stirring, to strong sulphuric acid, which must be cooled as soon as the reaction commences, to prevent decomposition. The reaction, which continues for upwards of twenty minutes, accompanied by evolution of sulphur dioxide, may be represented as follows:



The principal product of this reaction is a crystalline solid, of mild odor, which melts at 72-73° C., without decomposition or change in properties.

I propose to call this product tetraethyl tetrathio diphosphate, although other names may be equally appropriate. The following is a comparison of determined and theoretical constants of this product:

55

|                          | Determined | Theoretical |
|--------------------------|------------|-------------|
| Per cent sulphur.....    | 35.4       | 34.6        |
| Per cent phosphorus..... | 15.6       | 16.7        |
| Molecular weight.....    | 369.85     | 370.3       |

60

This compound is substantially insoluble in water, but dissolves in most organic solvents. I have found that it may be conveniently added to the mineral pulp in the molten condition, or in solution in alcohol, cresylic acid, sodium cresylate solution or other suitable solvent.

65

It is of course understood that I do not intend to limit myself to the use in flotation of the specific compound mentioned. A general formula of the type



75

expresses what I believe to be the constitution of the class of compounds which I intend to claim for use in flotation. In the general formula,  $R_1$ ,  $R_2$ ,  $R_3$  and  $R_4$  may represent any alkyl or aryl radicals or substituted derivatives thereof. The radicals may be all alike, as in the tetraethyl compound described in detail above; or some, or all, may be different. Methyl, propyl, phenyl and cresyl radicals may be mentioned, for example, as among those which can be represented by the symbols  $R_1$ ,  $R_2$ ,  $R_3$  and  $R_4$  above. While I believe that the above formula correctly represents the reaction product of an alkyl or aryl dithio phosphoric acid or its metallic salt with an oxidizing agent, it is understood that where I have used this formula in the claims such reaction product is indicated thereby.

80

Generally, these tetrathio diphospho organic compounds may be prepared through the reaction of any of the organic di-thio

85

90

95

100

phosphoric acids, or their metallic salts, with any suitable reagent that will effect the oxidation described. I may use any suitable oxidizing agent, such as sulphuric acid, the 5 halogens, hypohaloids, chromic acid, dichromates or permanganates. Typical results obtained by adding these reagents to a mineral ore pulp and subjecting the resulting mixture to flotation are tabulated as follows:

10 Utah Copper Company mill heading ground to a fine pulp and modified with burned lime and sodium cyanide was subjected to flotation in a Janney Laboratory machine. Cresylic acid was used at the rate of 15 .3 pounds per ton of ore and tetraethyl tetrathio diphosphate used at the rate of .05 lbs. in Test 1 and at the rate of .025 lbs. in Test 2.

| 20 | Test   | Heading        |                | Rougher<br>per cent<br>Cu | Tailing<br>per cent<br>Fe | Rougher<br>per cent<br>Cu | Concen-<br>trate per<br>cent Fe |
|----|--------|----------------|----------------|---------------------------|---------------------------|---------------------------|---------------------------------|
|    |        | Per cent<br>Cu | Per cent<br>Fe |                           |                           |                           |                                 |
| 25 | 1----- | :856           | 2.45           | 0.84                      | 1.85                      | 18.650                    | 14.90                           |
|    | 2----- | :856           | 2.45           | 0.89                      | 1.85                      | 22.585                    | 16.25                           |

30 I have found that these tetrathio diphospho organic compounds are effective flotation agents when mixed with a pulp so modified as to show either acid, alkaline or neutral reaction, and the resulting mixtures subjected to flotation operations.

I claim:

35 1. The improvement in the concentration of ore by froth flotation which comprises subjecting the ore in the form of a pulp to a froth flotation operation in the presence of the reaction product of diethyl dithio phosphoric acid with strong sulphuric acid.

40 2. The improvement in the concentration of ore by froth flotation which comprises subjecting the ore in the form of a pulp to a froth flotation operation in the presence of the reaction product of a metallic salt of diethyl dithio phosphoric acid with strong sulphuric acid.

45 3. The improvement in the concentration of ore by froth flotation which comprises subjecting the ore in the form of a pulp to a froth flotation operation in the presence of tetraethyl tetrathio diphosphate.

50 4. The improvement in the concentration of ore by froth flotation which comprises subjecting the ore in the form of a pulp to a froth flotation operation in the presence of a compound represented by the formula



65 in which  $\text{R}_1$ ,  $\text{R}_2$ ,  $\text{R}_3$  and  $\text{R}_4$  stand for any alkyl or aryl organic radicals or substituted derivatives thereof.

5 The improvement in the concentration of ore by froth flotation which comprises subjecting the ore in the form of a pulp to a froth flotation operation in the presence of an alkyl sulphur phosphorus compound containing two phosphorus atoms bonded through two intervening and interlinked sulphur atoms.

In testimony whereof, I have signed my name to this specification this 24th day of 75 October, 1928.

BENJAMIN L. JOHNSON.

80

85

90

95

100

105

110

115

120

125

130